# EUROPEAN PATENT SPECIFICATION

(11) **EP 4 470 635 B1**
(45) Date of publication and mention of the grant of the patent: **15.10.2025**
(21) Application number: 24173148.8
(22) Date of filing: 29.04.2024
(51) Int. Cl.: A63B 37/00

(54) **GOLF BALL**
GOLFBALL
BALLE DE GOLF

(30) Priority: 31.05.2023 JP 2023001871 U
(43) Date of publication of application: 04.12.2024
(62) Divisional of application: 25200197.9
(73) Proprietor: Sumitomo Rubber Industries, Ltd., Kobe-shi, Hyogo-ken 651-0072 (JP)
(72) Inventor: INOUE, Hidetaka, Kobe-shi, 651-0072 (JP); SAJIMA, Takahiro, Kobe-shi, 651-0072 (JP); FUKAO, Kaita, Kobe-shi, 651-0072 (JP)
(74) Representative: Manitz Finsterwald Patent- und Rechtsanwaltspartnerschaft mbB

(56) References cited:
- US-A1- 2016 303 430
- US-A1- 2017 028 261
- US-A1- 2017 173 398
- US-A1- 2021 138 307
- US-A1- 2022 280 840

## Description

### FIELD OF THE DISCLOSURE

The present disclosure relates to a golf ball, and relates to a golf ball reducing shots into an out-of-bounds (OB) area.

### DESCRIPTION OF THE RELATED ART

For an average golfer to make golf scores, it is important to reduce the number of shots into an out-of-bounds (OB) area on a driver shot. The reason why a driver shot goes OB includes a reason that the swing or hitting point is not stable, which is a reason in the player. On the other hand, a golf course is provided with a slope (downslope), and if a golf ball lands on the slope (downslope), it may roll too far and enter the OB area. Furthermore, the golf course is provided with obstacles such as trees to prevent OB, and if the golf ball flies too high, it may jump over the obstacles and enter the OB area.

Dimples are provided on a surface of a golf ball. The flight performance of the golf ball has been improved by improving the dimples.

For example, JP 2016-7369 A discloses a golf ball having a large number of dimples on a surface thereof, and satisfying the following mathematical formula (I): $1.320 \leq L 1 \leq 1.420$ wherein in the mathematical formula (I), L1 represents a ratio of a lift force coefficient CL1 which is measured under conditions of a Reynolds number of 1.290×10⁵ and a spin rate of 2820 rpm, relative to a lift force coefficient CL2 which is measured under conditions of a Reynolds number of 1.290×10⁵ and a spin rate of 1740 rpm.

US 2017 0173398 A1 discloses a golf ball comprising a golf ball body and a paint film formed on a surface of the golf ball body. The golf ball body comprises a spherical core, an intermediate layer and a cover. The paint film has a multi-layered construction composed of two or more layers and a difference between a 10% elastic modulus of an innermost layer of the paint film and a 10 % elastic modulus of an outermost layer of the paint film is 25 kgf/cm² or more.

### SUMMARY OF THE DISCLOSURE

An object of the present disclosure is to provide a golf ball having a high spin rate without an excess lift on the golf ball so that a maximum flying height is not high, thereby having a reduced number of shots into the OB area on a driver shot.

The present disclosure that has solved the above problem provides a golf ball comprising a spherical core, an intermediate layer positioned outside the spherical core, and an outermost cover positioned outside the intermediate layer and having a plurality of dimples formed thereon, wherein
a material hardness Hm (Shore D hardness) of the intermediate layer,
a material hardness Hc (Shore D hardness) of the outermost cover,
a thickness Tc (mm) of the outermost cover, and
a total lower volume Vi (mm³) of the plurality of dimples satisfy,
Vi>365 and (Hc/Tc)×(Hm/Vi)≤7.5, and wherein
a surface hardness in Shore C hardness of the spherical core < a surface hardness in Shore C hardness of the intermediate layer > a surface hardness in Shore C hardness of the golf ball is satisfied.

If the golf ball according to the present disclosure is configured as above, the spin rate on a driver shot is increased. If the spin rate of the golf ball on a driver shot is increased, the rolling distance of the golf ball becomes short even if the golf ball lands on a slope (downslope). As a result, the rolling of the golf ball into the OB area is reduced. On the other hand, a high spin rate on the golf ball creates an excess lift on the golf ball than intended, but in the golf ball according to the present disclosure, the dimples and the construction of the golf ball satisfy a specific relationship, so that the excess lift on the golf ball on a driver shot is suppressed. As a result, the excess lift on the golf ball is prevented, and the height on a driver shot can be lowered.

The present disclosure provides a golf ball that has a high spin rate without an excess lift on the golf ball so that a high maximum flying height is not high. The golf ball according to the present disclosure has a reduced number of shots into the out-of-bounds (OB) area on a driver shot.

### BRIEF DESCRIPTION OF THE DRAWINGS

Fig. 1 is a partially cutaway cross-sectional view showing a golf ball according to one embodiment of the present disclosure;
Fig. 2 is a front view of a dimple pattern formed on an outermost cover;
Fig. 3 is a plane view of a dimple pattern formed on an outermost cover; and
Fig. 4 is an enlarged sectional view of dimples formed on an outermost cover.

### DESCRIPTION OF THE PREFERRED EMBODIMENT

The present disclosure provides a golf ball comprising a spherical core, an intermediate layer positioned outside the spherical core, and an outermost cover positioned outside the intermediate layer and having a plurality of dimples formed thereon, wherein a material hardness Hm (Shore D hardness) of the intermediate layer, a material hardness Hc (Shore D hardness) of the outermost cover, a thickness Tc (mm) of the outermost cover, and a total lower volume Vi (mm³) of the plurality of dimples satisfy Vi>365 and (Hc/Tc)×(Hm/Vi)≤7.5, and wherein a surface hardness in Shore C hardness of the spherical core < a surface hardness in Shore C hardness of the intermediate layer > a surface hardness in Shore C hardness of the golf ball is satisfied.

### (Construction of golf ball)

The golf ball according to the present disclosure comprises a spherical core, an intermediate layer positioned outside of the spherical core, and an outermost cover positioned outside of the intermediate layer and having a plurality of dimples formed thereon.

Examples of the construction of the golf ball include a three-piece golf ball composed of a single-layered spherical core, an intermediate layer covering the spherical core, and an outermost cover covering the intermediate layer; and a multi-piece golf ball (a four-piece golf ball, a five-piece golf ball, or the like) composed of a single-layered spherical core, two or more intermediate layers covering the spherical core, and an outermost cover covering the intermediate layers.

The construction of the spherical core may be a single-layered construction, or a multi-layered construction, and the single-layered construction is preferable. The construction of the intermediate layer may be a single-layered construction, or a multi-layered construction composed of at least two layers.

The diameter of the spherical core is preferably 34.8 mm or more, more preferably 36.8 mm or more, and even more preferably 38.8 mm or more, and is preferably 42.2 mm or less, more preferably 41.8 mm or less, even more preferably 41.2 mm or less, and most preferably 40.8 mm or less. If the diameter of the spherical core falls within the above range, the golf ball has better flight distance performance or shot feeling.

When the spherical core has a diameter in the range from 34.8 mm to 42.2 mm, the compression deformation amount of the spherical core (shrinking amount of the spherical core along the compression direction) when applying a load from an initial load of 98 N to a final load of 1275 N to the spherical core is preferably 2.0 mm or more, more preferably 2.5 mm or more, and even more preferably 3.0 mm or more, and is preferably 5.0 mm or less, more preferably 4.5 mm or less, and even more preferably 4.0 mm or less. If the compression deformation amount falls within the above range, the shot feeling is better.

The surface hardness (Hs) of the spherical core is not particularly limited, but the surface hardness (Hs) is preferably 60 or more, more preferably 65 or more, and even more preferably 70 or more, and is preferably 95 or less, more preferably 90 or less, and even more preferably 85 or less in Shore C hardness. If the surface hardness (Hs) falls within the above range, better shot feeling is obtained.

The center hardness (Ho) of the spherical core is not particularly limited, but the center hardness (Ho) is preferably 45 or more, more preferably 47 or more, and even more preferably 49 or more, and is preferably 74 or less, more preferably 72 or less, and even more preferably 70 or less in Shore C hardness. If the center hardness (Ho) falls within the above range, better shot feeling is obtained.

The material hardness Hm of the intermediate layer composition constituting the intermediate layer is preferably 50 or more, more preferably 52 or more, and even more preferably 54 or more, and is preferably 73 or less, more preferably 72 or less, and even more preferably 70 or less in Shore D hardness. If the material hardness Hm is 50 or more, the flight distance is better due to the low spin rate on a driver shot, and if the material hardness Hm is 73 or less, better shot feeling is obtained when the golf ball is hit. It is noted that in case of comprising a plurality of intermediate layers, the material hardness of the intermediate layer composition constituting the outermost intermediate layer is adopted as the material hardness Hm.

The thickness Tm of the intermediate layer is preferably 0.8 mm or more, more preferably 0.9 mm or more, and even more preferably 1.0 mm or more, and is preferably 3.0 mm or less, more preferably 2.7 mm or less, and even more preferably 2.5 mm or less. If the thickness Tm is 0.8 mm or more, the durability is better, and if the thickness Tm is 3.0 mm or less, better shot feeling is obtained. It is noted that in case of comprising a plurality of intermediate layers, the total thickness of all the intermediate layers is adopted as the thickness Tm of the intermediate layer.

The material hardness Hc of the cover composition constituting the outermost cover is preferably 20 or more, more preferably 22 or more, and even more preferably 24 or more, and is preferably 40 or less, more preferably 39 or less, and even more preferably 38 or less in Shore D hardness. If the material hardness Hc is 20 or more, the spin rate on a driver shot is not excessively high and thus the flight distance performance is better, and if the material hardness Hc is 40 or less, the spin performance on an approach shot is better.

The thickness Tc of the outermost cover is preferably 0.4 mm or more, more preferably 0.5 mm or more, and even more preferably 0.6 mm or more, and is preferably 1.0 mm or less, more preferably 0.9 mm or less, and even more preferably 0.8 mm or less. If the thickness Tc is 0.4 mm or more, the spin performance on an approach shot is better, and if the thickness Tc is 1.0 mm or less, the spin rate on a driver shot is not excessively high and thus the flight distance performance is better.

The value (Hc/Tc) of the slab hardness Hc (Shore D) to the thickness Tc (mm) of the outermost cover is preferably 30 or more, more preferably 33 or more, and even more preferably 35 or more, and is preferably 75 or less, more preferably 72 or less, and even more preferably 70 or less. If the value (Hc/Tc) is 30 or more, the resilience performance is better, and if the value (Hc/Tc) is 75 or less, better shot feeling is obtained when the golf ball is hit.

### (Dimples)

The golf ball according to the present disclosure comprises an outermost cover having a plurality of dimples formed thereon. The dimples are concaves formed on the outermost cover. Next, the dimples formed on the outermost cover of the golf ball according to the present disclosure will be described with reference to the figures.

A golf ball 2 shown in Fig. 1 comprises a spherical core 4, an intermediate layer 6 covering the core 4, and an outermost cover 8 positioned outside the intermediate layer 6. The golf ball 2 has a plurality of dimples 10 on the surface thereof. Other portions than the dimples 10 on the surface of the golf ball 2 are lands 12. The golf ball 2 is provided with a paint layer and a mark layer on an outer side of the outermost cover 8, but these layers are not depicted.

As shown in Fig. 2 and Fig. 3, the outermost cover of the golf ball 2 has a plurality of dimples 10 formed on the surface. Each of the dimples 10 has a circle contour.

Fig. 4 shows a cross section of the golf ball 2 along a plane passing through the central point of the dimple 10 and the central point of the golf ball 2. The top-to-bottom direction in Fig. 4 is the depth direction of the dimple 10. In Fig. 4, a chain double-dashed line 14 indicates a virtual sphere. The surface of the virtual sphere 14 is the surface of the golf ball 2 when it is virtualized that no dimple 10 exists. The diameter of the virtual sphere 14 is equal to the diameter of the golf ball 2. The dimple 10 is recessed from the surface of the virtual sphere 14. The land 12 coincides with the surface of the virtual sphere 14. In the present embodiment, the cross-sectional shape of the dimple 10 is substantially a circular arc. The curvature radius of this circular arc is shown by a reference sign CR in Fig. 4.

In Fig. 4, an arrow Dm indicates the diameter of the dimple 10. The diameter Dm is a distance between one tangent point Ed and another tangent point Ed when a tangent line Tg traversing two sides of the dimple 10 is drawn. The tangent point Ed is also the edge of the dimple 10. The edge Ed defines the contour of the dimple 10.

In the present disclosure, the "volume of the dimple" means the volume of the portion surrounded by the surface of the dimple 10 and the surface of the virtual sphere including the contour of the dimple 10. The "volume of the dimple" is divided by a plane connecting intersection points Ed-Ed of the surface of the virtual sphere 14 with the surface of the dimple. The "upper volume of the dimple" is the volume of the dimple upper part surrounded by the surface of the virtual sphere 14 and the plane connecting the intersection points Ed-Ed of the surface of the dimple. The "lower volume of the dimple" is the volume of the dimple lower part surrounded by the plane connecting the intersection points Ed-Ed of the surface of the dimple and the surface of the dimple 10. The volume of the dimple is the sum of the upper volume and the lower volume. The "total volume V of the dimples" in the present disclosure is the sum of the volume of all the dimples. The "total upper volume Vo of the dimples" is the sum of the upper volume of all the dimples. The "total lower volume Vi of the dimples" is the sum of the lower volume of all the dimples. When the total upper volume of the dimples is Vo, and the total lower volume of the dimples is Vi, so V=Vo+Vi.

The total lower volume Vi of the plurality of dimples of the golf ball is more than 365 mm³, preferably 380 mm³ or more, more preferably 400 mm³ or more. If the total lower volume Vi is more than 365 mm³, the lift force that acts upon the golf ball is suppressed due to the backspin, and the excess lift on a driver shot is suppressed. The total lower volume Vi is preferably 500 mm³ or less, more preferably 495 mm³ or less, and even more preferably 490 mm³ or less. If the total lower volume Vi is 500 mm³ or less, the lift force that acts upon the golf ball on a driver shot is fully obtained, and the flight distance performance is better.

The diameter Dm of the dimple 10 is preferably 2.0 mm or more, more preferably 2.5 mm or more, and even more preferably 2.8 mm or more, and is preferably 6.0 mm or less, more preferably 5.5 mm or less, and even more preferably 5.0 mm or less. If the diameter Dm is 2.0 mm or more, the dimples easily contribute to the turbulent air flow, and if the diameter Dm is 6.0 mm or less, the nature of the golf ball that is substantially a spherical body can be kept.

The plurality of dimples may be a plurality of dimples with a single diameter, or a combination of dimples with various types of diameters. The golf ball 2 shown in Fig. 2 and Fig. 3 has five types of dimples, i.e. a dimple A with a diameter of 4.400 mm, a dimple B with a diameter of 4.285 mm, a dimple C with a diameter of 4.150 mm, a dimple D with a diameter of 3.875 mm, and a dimple E with a diameter of 3.000 mm.

In Fig. 4, a double ended arrow Dp1 indicates a first depth of the dimple 10. The first depth Dp1 is the distance between the deepest part of the dimple 10 and the surface of the virtual sphere 14.

The first depth Dp1 is preferably 0.15 mm or more, more preferably 0.17 mm or more, and even more preferably 0.20 mm or more, and is preferably 0.45 mm or less, more preferably 0.43 mm or less, and even more preferably 0.40 mm or less. If the first depth Dp1 is 0.15 mm or more, the lift force obtained by the dimples fully occurs, and if the first depth Dp1 is 0.45 mm or less, the nature of the golf ball that is substantially a spherical body can be kept.

In Fig. 4, a double ended arrow Dp2 indicates a second depth of the dimple 10. The second depth Dp2 is the distance between the deepest part of the dimple 10 and the tangent line Tg.

The second depth Dp2 is preferably 0.08 mm or more, more preferably 0.10 mm or more, and even more preferably 0.12 mm or more, and is preferably 0.30 mm or less, more preferably 0.28 mm or less, and even more preferably 0.26 mm or less. If the second depth Dp2 is 0.08 mm or more, the dimples easily contribute to the turbulent air flow, and if the second depth Dp2 is 0.30 mm or less, the lift force obtained by the dimples is not excessively great, and the flight distance performance on a driver shot is better.

The area A of the dimple 10 is the area of a region surrounded by the contour of the dimple 10 when the central point of the golf ball 2 is viewed at infinity. In the case that the dimple 10 has a circular shape, the area A is calculated by the following mathematical formula. $A = π \times {\left(Dm/2\right)}^{2}$

In the golf ball 2 shown in Fig. 2 and Fig. 3, the area of the dimple A is 15.21 mm², the area of the dimple B is 14.42 mm², the area of the dimple C is 13.53 mm², the area of the dimple D is 11.79 mm², and the area of the dimple E is 7.07 mm².

The ratio (total areas of dimples/surface area of virtual sphere) of the sum of the areas A of all the dimples 10 to the surface area of the virtual sphere 14 is referred to as an occupation ratio So. The occupation ratio So is preferably 70% or more, more preferably 75% or more, and even more preferably 80% or more, and is preferably 95% or less, more preferably 92% or less, and even more preferably 90% or less. If the occupation ratio So falls within the above range, the effect of the turbulence by the dimples is greater.

The number of the dimples can be appropriately adjusted depending on the diameter or occupation ratio of the dimples. It is noted that from the viewpoint of the occupation ratio or the function of the respective dimple, the total number of the dimples 10 is preferably 250 or more, more preferably 280 or more, and even more preferably 300 or more, and is preferably 450 or less, more preferably 410 or less, and even more preferably 390 or less.

The golf ball according to the present disclosure satisfies (Hc/Tc)×(Hm/Vi)≤7.5. The value (Hc/Tc)×(Hm/Vi) is preferably 3.0 or more, more preferably 3.3 or more, and even more preferably 3.5 or more, and is preferably 7.2 or less, more preferably 7.0 or less. If the value (Hc/Tc)×(Hm/Vi) falls within the above range, the launch angle is small on a driver shot and the lift force due to the dimples is suppressed, thus the maximum flying height is suppressed.

The value (Hm/Vi) is preferably 0.08 or more, more preferably 0.09 or more, and even more preferably 0.10 or more, and is preferably 0.22 or less, more preferably 0.20 or less, and even more preferably 0.18 or less. If the value (Hm/Vi) falls within the above range, lowering in the spin rate on a driver shot and the turbulence by the dimples fully occur, and thus the flight distance performance is better.

The golf ball according to the present disclosure preferably satisfies the surface hardness Hs (Shore C hardness) of the spherical core < the surface hardness Hms (Shore C hardness) of the intermediate layer > the surface hardness Hcs (Shore C hardness) of the golf ball.

The difference (Hms-Hcs) between the surface hardness Hms of the intermediate layer and the surface hardness Hcs of the golf ball is preferably more than 0, more preferably 2 or more, and even more preferably 4 or more in Shore C hardness. If the difference (Hms-Hcs) is more than 0, the spin performance on an approach shot is better since the deformation of the cover when the golf ball is hit is greater. It is noted that the upper limit of the difference (Hms-Hcs) is not particularly limited, but it is about 20 in Shore C hardness.

The difference (Hms-Hs) between the surface hardness Hms of the intermediate layer and the surface hardness Hs of the spherical core is preferably more than 0, more preferably 2 or more, and even more preferably 4 or more in Shore C hardness. If the difference (Hms-Hs) is more than 0, the whole intermediate layer-covering spherical body having the intermediate layer formed on the surface of the spherical core has a greater outer-hard and inner-soft degree, and the spin rate on a driver shot can be suppressed.

The golf ball according to the present disclosure preferably has a diameter ranging from 40 mm to 45 mm. In light of satisfying the regulation of US Golf Association (USGA), the diameter is particularly preferably 42.67 mm or more. In light of prevention of air resistance, the diameter is more preferably 44 mm or less, and particularly preferably 42.80 mm or less. In addition, the golf ball according to the present disclosure preferably has a mass of 40 g or more and 50 g or less. In light of obtaining greater inertia, the mass is more preferably 44 g or more, and particularly preferably 45.00 g or more. In light of satisfying the regulation of USGA, the mass is particularly preferably 45.93 g or less.

When the golf ball has a diameter in the range of from 40 mm to 45 mm, the compression deformation amount (shrinking amount along the compression direction) of the golf ball when applying a load from an initial load of 98 N to a final load of 1275 N to the golf ball is preferably 2.0 mm or more, more preferably 2.1 mm or more, and even more preferably 2.2 mm or more, and is preferably 3.0 mm or less, more preferably 2.9 mm or less, and even more preferably 2.8 mm or less. If the compression deformation amount falls within the above range, the golf ball has better shot feeling.

Next, the materials for forming the constituent members of the golf ball according to the present disclosure will be explained.

### (Core composition)

The spherical core of the golf ball according to the present disclosure is preferably formed from a rubber composition (hereinafter sometimes referred to as "core rubber composition") containing (a) a base rubber, (b) an α,β-unsaturated carboxylic acid having 3 to 8 carbon atoms and/or a metal salt thereof as a co-crosslinking agent, and (c) a crosslinking initiator.

As (a) the base rubber, a natural rubber and/or a synthetic rubber can be used. For example, a polybutadiene rubber, a natural rubber, a polyisoprene rubber, a styrene polybutadiene rubber, or an ethylene-propylene-diene rubber (EPDM) can be used. These rubbers may be used solely, or at least two of these rubbers may be used in combination.

(b) The α,β-unsaturated carboxylic acid having 3 to 8 carbon atoms and/or the metal salt thereof is blended as a co-crosslinking agent in the rubber composition, and has an action of crosslinking a rubber molecule by graft polymerization to a base rubber molecular chain.

Examples of the α,β-unsaturated carboxylic acid having 3 to 8 carbon atoms include acrylic acid, methacrylic acid, fumaric acid, maleic acid and crotonic acid.

Examples of the metal ion constituting the metal salt of the α,β-unsaturated carboxylic acid having 3 to 8 carbon atoms include a monovalent metal ion such as sodium, potassium and lithium; a divalent metal ion such as magnesium, calcium, zinc, barium and cadmium; a trivalent metal ion such as aluminum; and other metal ions such as tin and zirconium. The above metal component may be used solely or as a mixture of at least two of them. Among them, the divalent metal ion such as magnesium, calcium, zinc, barium and cadmium is preferably used as the metal component. This is because if the divalent metal salt of the α,β-unsaturated carboxylic acid having 3 to 8 carbon atoms is used, a metal crosslinking easily generates between the rubber molecules. Especially, as the divalent metal salt, zinc acrylate is preferable, because zinc acrylate enhances the resilience of the obtained golf ball. It is noted that the α,β-unsaturated carboxylic acid having 3 to 8 carbon atoms and/or the metal salt thereof may be used solely or as a mixture of at least two of them.

The amount of (b) the α,β-unsaturated carboxylic acid having 3 to 8 carbon atoms and/or the metal salt thereof may be appropriately adjusted depending on the desired hardness of the spherical core. For example, the amount of the component (b) is preferably 15 parts by mass or more, more preferably 20 parts by mass or more, and is preferably 50 parts by mass or less, more preferably 40 parts by mass or less, with respect to 100 parts by mass of (a) the base rubber.

(c) The crosslinking initiator is blended to crosslink (a) the base rubber component. As (c) the crosslinking initiator, an organic peroxide is suitable. Specific examples of the organic peroxide include dicumyl peroxide, 1,1-bis(t-butylperoxy)-3,3,5-trimethylcyclohexane, 2,5-dimethyl-2,5-di(t-butylperoxy) hexane and di-t-butyl peroxide. These organic peroxides may be used solely or as a mixture of at least two of them. Among them, dicumyl peroxide is preferably used.

The amount of (c) the crosslinking initiator may be appropriately adjusted depending on the desired hardness of the spherical core. For example, the amount of (c) the crosslinking initiator is preferably 0.2 part by mass or more, more preferably 0.4 part by mass or more, and is preferably 5.0 parts by mass or less, more preferably 2.5 parts by mass or less, and even more preferably 1.0 part by mass or less, with respect to 100 parts by mass of (a) the base rubber.

In the case that the co-crosslinking agent of the rubber composition consists of the α,β-unsaturated carboxylic acid having 3 to 8 carbon atoms, the rubber composition preferably further contains (d) a metal compound. This is because if the α,β-unsaturated carboxylic acid having 3 to 8 carbon atoms is neutralized with the metal compound in the rubber composition, substantially the same effect as using the metal salt of the α,β-unsaturated carboxylic acid having 3 to 8 carbon atoms as the co-crosslinking agent is provided. In addition, in the case that the α,β-unsaturated carboxylic acid having 3 to 8 carbon atoms and the metal salt thereof are used in combination as the co-crosslinking agent, (d) the metal compound may be used.

(d) The metal compound is not particularly limited, as long as it can neutralize (b) the α,β-unsaturated carboxylic acid having 3 to 8 carbon atoms in the rubber composition. Examples of (d) the metal compound include a metal hydroxide such as magnesium hydroxide, zinc hydroxide, calcium hydroxide, sodium hydroxide, lithium hydroxide, potassium hydroxide, and copper hydroxide; a metal oxide such as magnesium oxide, calcium oxide, zinc oxide, and copper oxide; and a metal carbonate such as magnesium carbonate, zinc carbonate, calcium carbonate, sodium carbonate, lithium carbonate, and potassium carbonate. As (d) the metal compound, the divalent metal compound is preferable, the zinc compound is more preferable. This is because the divalent metal compound reacts with the α,β-unsaturated carboxylic acid having 3 to 8 carbon atoms to form a metal crosslinking. (d) The metal compound may be used solely, or at least two of them may be used in combination.

The rubber composition may further contain (e) an organic sulfur compound. (e) The organic sulfur compound enhances the resilience of the spherical core. (e) The organic sulfur compound is not particularly limited, as long as it is an organic compound having a sulfur atom in the molecule thereof. Examples of (e) the organic sulfur compound include an organic compound having a thiol group (-SH) or a polysulfide bond having 2 to 4 sulfur atoms (-S-S-, -S-S-S-, or -S-S-S-S-), and a metal salt thereof (-SM, -S-M-S- or the like; M is a metal atom). (e) The organic sulfur compound may be used solely or as a mixture of at least two of them.

Examples of (e) the organic sulfur compound include thiophenols, thionaphthols, polysulfides, thiurams, thiocarboxylic acids, dithiocarboxylic acids, sulfenamides, dithiocarbamates, and thiazoles. As the organic sulfur compound, diphenyl disulfides (e.g. diphenyl disulfide, bis(pentabromophenyl) disulfide), thiophenols, and thionaphthols (e.g. 2-thionaphthol) can be suitably used.

The amount of (e) the organic sulfur compound may be appropriately adjusted depending on the desired resilience performance of the spherical core. For example, the amount of (e) the organic sulfur compound is preferably 0.05 part by mass or more, more preferably 0.1 part by mass or more, and is preferably 5.0 parts by mass or less, more preferably 3.0 parts by mass or less, with respect to 100 parts by mass of (a) the base rubber.

The rubber composition may further contain (f) a carboxylic acid and/or a metal salt thereof. As (f) the carboxylic acid and/or the metal salt thereof, a carboxylic acid having 1 to 30 carbon atoms and/or a metal salt thereof is preferable. As the carboxylic acid, an aliphatic carboxylic acid (a saturated fatty acid or an unsaturated fatty acid), or an aromatic carboxylic acid (benzoic acid) can be used. The amount of (f) the carboxylic acid and/or the metal salt thereof is preferably 1 part by mass or more and 40 parts by mass or less with respect to 100 parts by mass of the base rubber.

The rubber composition may further contain an additive such as a filler for adjusting weight or the like, an antioxidant, a peptizing agent, and a softener, where necessary.

The filler blended in the rubber composition is mainly used as a weight adjusting agent for adjusting the weight of the golf ball obtained as a final product, and may be blended where necessary. Examples of the filler include an inorganic filler such as barium sulfate, calcium carbonate, magnesium oxide, tungsten powder, and molybdenum powder.

The rubber composition can be obtained by kneading (a) the base rubber, (b) the α,β-unsaturated carboxylic acid having 3 to 8 carbon atoms and/or the metal salt thereof, (c) the crosslinking initiator, and the other optional components. The kneading method is not particularly limited. For example, the kneading can be conducted with a conventional kneading machine such as a kneading roll, a banbury mixer and a kneader.

The spherical core can be molded, for example, by heat pressing the core rubber composition. The molding conditions for heat pressing the core rubber composition may be determined appropriately depending on the rubber composition. Generally, the heat pressing is preferably carried out at a temperature of 130 °C to 200 °C for 10 to 60 minutes, or carried out in a two-step heating of heating at a temperature of 130 °C to 150 °C for 20 to 40 minutes followed by heating at a temperature of 160 °C to 180 °C for 5 to 15 minutes.

### (Cover composition and intermediate layer composition)

The golf ball according to the present disclosure has an intermediate layer covering the spherical core. The intermediate layer is preferably formed from an intermediate layer composition containing a resin component.

The golf ball according to the present disclosure has an outermost cover positioned outside of the intermediate layer. The outermost cover is preferably formed from a cover composition containing a resin component.

Examples of the resin component used in the resin composition forming the outermost cover and the intermediate layer include an ionomer resin, a urethane resin (a thermoplastic polyurethane elastomer or a thermosetting polyurethane elastomer), a thermoplastic styrene elastomer, a thermoplastic polyamide elastomer, and a thermoplastic polyester elastomer.

Examples of the ionomer resin include a binary ionomer resin prepared by neutralizing at least a part of carboxyl groups in a binary copolymer composed of an olefin and an α, β-unsaturated carboxylic acid having 3 to 8 carbon atoms with a metal ion, a ternary ionomer resin prepared by neutralizing at least a part of carboxyl groups in a ternary copolymer composed of an olefin, an α, β-unsaturated carboxylic acid having 3 to 8 carbon atoms and an α, β-unsaturated carboxylic acid ester with a metal ion, and a mixture of those.

Examples of the binary ionomer resin include Himilan (registered trademark) 1555 (Na), 1557 (Zn), 1605 (Na), 1706 (Zn), 1707 (Na), AM7311 (Mg), AM7329 (Zn), AM7337 (available from Dow-Mitsui Polychemicals Co., Ltd.); Surlyn (registered trademark) 8945 (Na), 9945 (Zn), 8140 (Na), 8150 (Na), 9120 (Zn), 9150 (Zn), 6910 (Mg), 6120 (Mg), 7930 (Li), 7940 (Li), AD8546 (Li) (available from E.I. du Pont de Nemours and Company); and lotek (registered trademark) 8000 (Na), 8030 (Na), 7010 (Zn), 7030 (Zn) (available from ExxonMobil Chemical Corporation).

Examples of the ternary ionomer resin include Himilan AM7327 (Zn), 1855 (Zn), 1856 (Na), AM7331 (Na) (available from Dow-Mitsui Polychemicals Co., Ltd.); Surlyn 6320 (Mg), 8120 (Na), 8320 (Na), 9320 (Zn), 9320W (Zn), HPF1000 (Mg), HPF2000 (Mg) (available from E.I. du Pont de Nemours and Company); and lotek7510 (Zn), 7520 (Zn) (available from ExxonMobil Chemical Corporation). It is noted that Na, Zn, Li, Mg or the like described in the parentheses after the trade names of the ionomer resin indicate metal ion type for neutralizing the ionomer resin.

The thermoplastic polyurethane elastomer has a urethane bond in the molecule. The urethane bond may be formed by a reaction between a polyol and a polyisocyanate. The polyol which is the raw material for the urethane bond has a plurality of hydroxy groups, and a low molecular weight polyol or a high molecular weight polyol may be used.

Specific examples of the thermoplastic polyurethane elastomer include Elastollan (registered trademark) NY80A, NY84A, NY88A, NY95A, ET885, ET890 (available from BASF Japan Ltd.).

As the thermoplastic styrene based elastomer, a styrene block-containing thermoplastic elastomer can be suitably used. The styrene block-containing thermoplastic elastomer has a polystyrene block as a hard segment, and a soft segment.

The styrene block-containing thermoplastic elastomer includes a styrenebutadiene-styrene block copolymer (SBS), a styrene-isoprene-styrene block copolymer (SIS), a styrene-isoprene-butadiene-styrene block copolymer (SIBS), a hydrogenated product of SBS, a hydrogenated product of SIS, and a hydrogenated product of SIBS. Examples of the hydrogenated product of SBS include a styrene-ethylene-butylene-styrene block copolymer (SEBS). Examples of the hydrogenated product of SIS include a styrene-ethylene-propylene-styrene block copolymer (SEPS). Examples of the hydrogenated product of SIBS include a styrene-ethylene-ethylene-propylene-styrene block copolymer (SEEPS).

Examples of the thermoplastic styrene based elastomer include TEFABLOC T3221C, T3339C, SJ4400N, SJ5400N, SJ6400N, SJ7400N, SJ8400N, SJ9400N, SR04 (available from Mitsubishi Chemical Corporation).

The cover composition constituting the outermost cover preferably contains the polyurethane and/or the ionomer resin as the resin component, and particularly preferably contains the polyurethane as the resin component. If the outermost cover contains the polyurethane as the resin component, the bite of the outermost cover into the club face on a driver shot is greater, and thus the spin rate is easily increased.

In the case that the cover composition contains the polyurethane as the resin component, the amount of the polyurethane in the resin component is preferably 50 mass % or more, more preferably 60 mass % or more, and even more preferably 70 mass % or more. The resin component of the cover composition may consist of the polyurethane (preferably the thermoplastic polyurethane elastomer).

In the case that the cover composition contains the ionomer resin as the resin component, the amount of the ionomer resin in the resin component is preferably 50 mass % or more, more preferably 60 mass % or more, and even more preferably 70 mass % or more. When the ionomer resin is contained, it is also preferable that the thermoplastic styrene elastomer is used in combination.

The intermediate layer composition preferably contains the ionomer resin as the resin component. When the ionomer resin is contained, it is also preferable that the thermoplastic styrene elastomer is used in combination. The amount of the ionomer resin in the resin component of the intermediate layer composition is preferably 50 mass % or more, more preferably 60 mass % or more, and even more preferably 70 mass % or more.

The outermost cover composition and the intermediate layer composition may contain a pigment component such as a white pigment (e.g. titanium oxide), a blue pigment and a red pigment, a weight adjusting agent such as zinc oxide, calcium carbonate and barium sulfate, a dispersant, an antioxidant, an ultraviolet absorber, a light stabilizer, a fluorescent material or fluorescent brightener, or the like, in addition to the above resin component.

The amount of the white pigment (e.g. titanium oxide) is preferably 0.5 part by mass or more, more preferably 1 part by mass or more, and is preferably 10 parts by mass or less, more preferably 8 parts by mass or less, with respect to 100 parts by mass of the base resin constituting the outermost cover. If the amount of the white pigment is 0.5 part by mass or more, it is possible to impart the opacity to the cover. In addition, if the amount of the white pigment is 10 parts by mass or less, the obtained cover has better durability.

The method for forming the intermediate layer is not particularly limited, and examples thereof include a method which comprises molding the intermediate layer composition into a hemispherical half-shell in advance, covering the spherical core with two of the half-shells, and performing compression molding; and a method which comprises injection molding the intermediate layer composition directly onto the spherical core to cover the spherical core.

Examples of the method for molding the cover include a method which comprises molding the cover composition into a hollow shell, covering the spherical body (the spherical body having the spherical core and the intermediate layer) with a plurality of the hollow shells, and performing compression molding (preferably a method which comprises molding the cover composition into a hollow half-shell, covering the spherical body with two of the half-shells, and performing compression molding); and a method which comprises injection molding the cover composition directly onto the spherical body.

The golf ball body having the cover formed thereon is ejected from the mold, and is preferably subjected to surface treatments such as deburring, cleaning and sandblast where necessary.

In addition, if desired, a paint film or a mark may be formed. The thickness of the paint film is not particularly limited, and is preferably 5 µm or more, more preferably 6 µm or more, and even more preferably 7 µm or more, and is preferably 50 µm or less, more preferably 40 µm or less, and even more preferably 30 µm or less. If the thickness of the paint film is 5 µm or more, the paint film is hard to wear off even if the golf ball is used continuously, and if the thickness of the paint film is 50 µm or less, the dimple effect is fully obtained. It is noted that the effect of the present disclosure is not impaired since the paint film is very thin.

### EXAMPLES

Next, the present disclosure will be described in detail by way of examples. However, the present disclosure is not limited to the examples described below. The subject-matter of the present invention concerns a golf ball according to claim 1. Preferred embodiments are the subject of dependent claims.

### [Evaluation method]

### (1) Material (slab) hardness (Shore D hardness)

Sheets with a thickness of about 2 mm were produced by injection molding the intermediate layer composition or cover composition. The sheets were stored at a temperature of 23 °C for two weeks. At least three of these sheets were stacked on one another so as not to be affected by the measuring substrate on which the sheets were placed, and the hardness of the stack was measured with an automatic hardness tester (Digitest II, available from Bareiss company) using a testing device of "Shore D".

### (2) Compression deformation amount (mm)

The compression deformation amount was measured with a YAMADA type compression tester "SCH". The golf ball or spherical core was placed on a metal rigid plate of the tester. A metal cylinder slowly fell toward the golf ball or spherical core. The golf ball or spherical core sandwiched between the bottom of the cylinder and the rigid plate deformed. The travelling distance of the cylinder when applying a load from an initial load of 98 N to a final load of 1275 N to the golf ball or spherical core was measured. The compression deformation amount (mm) is the travelling distance. The travelling speed of the cylinder before applying the initial load was 0.83 mm/s. The travelling speed of the cylinder when applying the load from the initial load to the final load was 1.67 mm/s.

### (3) Core hardness distribution (Shore C hardness)

The hardness measured at the surface portion of the core was adopted as the surface hardness of the core. The hardness was measured with an automatic hardness tester (Digitest II, available from Bareiss company) using a testing device of "Shore C".

### (4) Surface hardness of golf ball and surface hardness of intermediate layer

The hardness measured at the land on the surface portion of the golf ball was adopted as the surface hardness of the golf ball. In addition, the hardness measured at the surface portion of the intermediate layer-covering spherical body having the intermediate layer formed on the surface of the spherical core was adopted as the surface hardness of the intermediate layer. Each hardness was measured at four points and the average value thereof was calculated. The hardness was measured with an automatic hardness tester (Digitest II, available from Bareiss company) using a testing device of "Shore C".

### (4) Flight distance (m) on driver shot

A driver (trade name "XXIO12", Shaft hardness: S, Loft angle: 10.5°, available from Sumitomo Rubber Industries, Ltd.) was installed on a swing machine available from Golf Laboratories, Inc. The hitting point was set at the face center. The golf ball was hit under a condition of a head speed of 40 m/sec, and the spin rate (rpm) and launch angle (°) right after hitting the golf ball and the maximum flying height (mm) were measured. The measurement was conducted twelve times for each golf ball, and the average value of the obtained data was adopted as the measurement value for that golf ball. The spin rate and the launch angle were measured by continuously taking a sequence of photographs right after hitting the golf ball. The maximum flying height was measured with a launch monitor "TRACK MAN 4" available from TRACK MAN Golf.

### [Production of golf ball]

### (1) Preparation of core composition

According to the formulation shown in Table 1, the materials were kneaded with a kneading roll to obtain the core composition.

**Table 1**

| Core composition No. | | A |
|---|---|---|
| Formulation (parts by mass) | Polybutadiene | 100 |
| | Zinc acrylate | 30.1 |
| | Zinc oxide | 5 |
| | Barium sulfate | Appropriate amount^{*1)} |
| | bis(pentabromophenyl) disulfide | 0.4 |
| | Dicumyl peroxide | 0.7 |

| | | |
|---|---|---|
| *1) The amount of barium sulfate was adjusted such that the golf balls had a mass of 45.3 g. | | |

The materials used in Table 1 are shown as follows.
Polybutadiene: "BR-730" available from JSR Corporation
Zinc acrylate: "ZN-DA90S" available from Nisshoku Techno Fine Chemical Co., Ltd.
Zinc oxide: "Ginrei R" available from Toho Zinc Co., Ltd.
Barium sulfate: "Barium sulfate BD" available from Sakai Chemical Industry Co., Ltd.
Bis(pentabromophenyl) disulfide: available from Kawaguchi Chemical Industry Co., Ltd.
Dicumyl peroxide: "Percumyl (registered trademark) D" available from NOF Corporation

### (2) Preparation of intermediate layer composition

According to the formulations shown in Table 2, the materials were extruded with a twin-screw kneading type extruder to prepare the intermediate layer compositions in a pellet form.

**Table 2**

| Intermediate layer composition No. | | a | b | c | d |
|---|---|---|---|---|---|
| Formulation (parts by mass) | Surlyn 8150 | - | 50 | - | - |
| | Himilan 1605 | 50 | - | 47 | - |
| | Himilan AM7329 | 50 | 50 | 50 | - |
| | Himilan 1555 | - | - | - | 45 |
| | Himilan 1557 | - | - | - | 45 |
| | TEFABLOC T3221C | - | - | 3 | 10 |
| | Titanium dioxide | 4 | 4 | 4 | 4 |
| Hardness (Shore D) | | 66 | 68 | 63 | 55 |

| | | | | | |
|---|---|---|---|---|---|
| Surlyn (registered trademark) 8150: sodium ion neutralized ethylene-methacrylic acid copolymer ionomer resin available from E.I. du Pont de Nemours and Company Himilan (registered trademark) 1605: sodium ion neutralized ethylene-methacrylic acid copolymer ionomer resin available from Dow-Mitsui Polychemicals Co., Ltd. Himilan (registered trademark) AM7329: sodium ion neutralized ethylene-methacrylic acid copolymer ionomer resin available from Dow-Mitsui Polychemicals Co., Ltd. Himilan (registered trademark) 1555: sodium ion neutralized ethylene-methacrylic acid copolymer ionomer resin available from Dow-Mitsui Polychemicals Co., Ltd. Himilan (registered trademark) 1557: zinc ion neutralized ethylene-methacrylic acid copolymer ionomer resin available from Dow-Mitsui Polychemicals Co., Ltd. TEFABLOC T3221C: thermoplastic styrene based elastomer available from Mitsubishi Chemical Corporation Titanium dioxide: A-220 available from Ishihara Sangyo Kaisha, Ltd. | | | | | |

### (3) Preparation of cover composition

According to the formulations shown in Table 3, the materials were extruded with a twin-screw kneading type extruder to prepare the cover compositions in a pellet form.

**Table 3**

| Cover composition No. | | e | f | 9 | h | i |
|---|---|---|---|---|---|---|
| | Elastollan NY80A | 100 | - | - | - | - |
| | Elastollan NY84A | - | 100 | - | - | - |
| | Elastollan NY88A | - | - | 100 | 50 | - |
| | Elastollan NY95A | - | - | - | 50 | - |
| Formulation (parts by mass) | Himilan 1555 | - | - | - | - | 41 |
| | Himilan 1557 | - | - | - | - | 41 |
| | TEFABLOC T3221C | - | - | - | - | 18 |
| | TINUVIN 770 | 0.2 | 0.2 | 0.2 | 0.2 | 0.2 |
| | Titanium dioxide | 4 | 4 | 4 | 4 | 4 |
| Hardness (Shore D) | | 27 | 31 | 36 | 40 | 50 |

| | | | | | | |
|---|---|---|---|---|---|---|
| Elastollan (registered trademark) NY80A: thermoplastic polyurethane elastomer available from BASF Japan Ltd. Elastollan (registered trademark) NY84A: thermoplastic polyurethane elastomer available from BASF Japan Ltd. Elastollan (registered trademark) NY88A: thermoplastic polyurethane elastomer available from BASF Japan Ltd. Elastollan (registered trademark) NY95A: thermoplastic polyurethane elastomer available from BASF Japan Ltd. TINUVIN (registered trademark) 770: hindered amine based light stabilizer available from BASF Japan Ltd. Himilan (registered trademark) 1555: sodium ion neutralized ethylene-methacrylic acid copolymer ionomer resin available from Dow-Mitsui Polychemicals Co., Ltd. Himilan (registered trademark) 1557: zinc ion neutralized ethylene-methacrylic acid copolymer ionomer resin available from Dow-Mitsui Polychemicals Co., Ltd. TEFABLOC T3221C: thermoplastic styrene based elastomer available from Mitsubishi Chemical Corporation Titanium dioxide: A-220 available from Ishihara Sangyo Kaisha, Ltd. | | | | | | |

### (4) Production of core

The core compositions shown in Table 1 were heat-pressed in upper and lower molds, each having a hemispherical cavity, at a temperature of 155 °C for 20 minutes to produce the spherical cores. It is noted that barium sulfate was added in an appropriate amount such that the obtained golf balls had a mass of 45.3 g.

### (5) Formation of intermediate layer and cover

The intermediate layer compositions were injection molded on the spherical cores to obtain the intermediate layer-covering spherical bodies. The obtained intermediate layer-covering spherical bodies were charged into a final mold provided with a plurality of pimples on the cavity surface. Half shells were obtained from the cover composition by a compression molding method. The intermediate layer-covering spherical bodies charged into the final mold were covered with two of the half shells to obtain the golf balls having an outermost cover on which a plurality of dimples with a reversed shape of the pimple shape on the cavity surface were formed. The specifications of the dimples formed on the outermost cover are shown in Tables 4 to 6. The evaluation results regarding the obtained golf balls are shown in Tables 7 to 8.

**Table 4**

| Dimple pattern | Type | Number | Diameter | Depth Dp1 | Depth Dp2 | Curvature CR | Lower volume | Total lower volume |
|---|---|---|---|---|---|---|---|---|
| | | | (mm) | (mm) | (mm) | (mm) | (mm³) | Vi (mm³) |
| I | A | 60 | 4.400 | 0.2356 | 0.1219 | 19.9 | 0.93 | 56 |
| | B | 158 | 4.285 | 0.2297 | 0.1219 | 18.9 | 0.88 | 139 |
| | C | 72 | 4.150 | 0.2230 | 0.1219 | 17.7 | 0.83 | 59 |
| | D | 36 | 3.875 | 0.2100 | 0.1219 | 15.5 | 0.72 | 26 |
| | E | 12 | 3.000 | 0.1747 | 0.1219 | 9.3 | 0.43 | 5 |
| II | A | 60 | 4.400 | 0.2526 | 0.1389 | 17.5 | 1.06 | 63 |
| | B | 158 | 4.285 | 0.2467 | 0.1389 | 16.6 | 1.00 | 158 |
| | C | 72 | 4.150 | 0.2400 | 0.1389 | 15.6 | 0.94 | 68 |
| | D | 36 | 3.875 | 0.2270 | 0.1389 | 13.6 | 0.82 | 30 |
| | E | 12 | 3.000 | 0.1917 | 0.1389 | 8.2 | 0.49 | 6 |
| III | A | 60 | 4.400 | 0.2696 | 0.1559 | 15.6 | 1.19 | 71 |
| | B | 158 | 4.285 | 0.2637 | 0.1559 | 14.8 | 1.13 | 178 |
| | C | 72 | 4.150 | 0.2570 | 0.1559 | 13.9 | 1.06 | 76 |
| | D | 36 | 3.875 | 0.2440 | 0.1559 | 12.1 | 0.92 | 33 |
| | E | 12 | 3.000 | 0.2087 | 0.1559 | 7.3 | 0.55 | 7 |

**Table 5**

| Dimple pattern | Type | Number | Diameter | Depth Dp1 | Depth Dp2 | Curvature | Lower volume | Total lower volume |
|---|---|---|---|---|---|---|---|---|
| | | | (mm) | (mm) | (mm) | (mm) | (mm³) | Vi (mm3) |
| IV | A | 60 | 4.400 | 0.2866 | 0.1729 | 14.1 | 1.32 | 79 |
| | B | 158 | 4.285 | 0.2807 | 0.1729 | 13.4 | 1.25 | 197 |
| | C | 72 | 4.150 | 0.2740 | 0.1729 | 12.5 | 1.17 | 84 |
| | D | 36 | 3.875 | 0.2610 | 0.1729 | 10.9 | 1.02 | 37 |
| | E | 12 | 3.000 | 0.2257 | 0.1729 | 6.6 | 0.61 | 7 |
| V | A | 60 | 4.400 | 0.3036 | 0.1899 | 12.8 | 1.45 | 87 |
| | B | 158 | 4.285 | 0.2977 | 0.1899 | 12.2 | 1.37 | 217 |
| | C | 72 | 4.150 | 0.2910 | 0.1899 | 11.4 | 1.29 | 93 |
| | D | 36 | 3.875 | 0.2780 | 0.1899 | 10.0 | 1.12 | 40 |
| | E | 12 | 3.000 | 0.2427 | 0.1899 | 6.0 | 0.67 | 8 |
| VI | A | 60 | 4.400 | 0.3206 | 0.2069 | 11.8 | 1.58 | 95 |
| | B | 158 | 4.285 | 0.3147 | 0.2069 | 11.2 | 1.50 | 236 |
| | C | 72 | 4.150 | 0.3080 | 0.2069 | 10.5 | 1.40 | 101 |
| | D | 36 | 3.875 | 0.2950 | 0.2069 | 9.2 | 1.22 | 44 |
| | E | 12 | 3.000 | 0.2597 | 0.2069 | 5.5 | 0.74 | 9 |

**Table 6**

| Dimple pattern No. | I | II | III | IV | V | VI |
|---|---|---|---|---|---|---|
| Front view | Fig. 2 | Fig. 2 | Fig. 2 | Fig. 2 | Fig. 2 | Fig. 2 |
| Plane view | Fig. 3 | Fig. 3 | Fig. 3 | Fig. 3 | Fig. 3 | Fig. 3 |
| Total number | 338 | 338 | 338 | 338 | 338 | 338 |
| Total lower volume Vi (mm³) | 285 | 325 | 365 | 405 | 445 | 485 |
| Occupation ratio (%) | 81.6 | 81.6 | 81.6 | 81.6 | 81.6 | 81.6 |

**Table 7**

| Golf ball No. | | 1 | 2 | 3 | 4 | 5 |
|---|---|---|---|---|---|---|
| Core | Formulation No. | A | A | A | A | A |
| | Diameter (mm) | 39.5 | 39.5 | 39.5 | 39.5 | 39.1 |
| | Surface hardness Hs (Shore C) | 81.3 | 81.3 | 81.3 | 81.3 | 81 |
| | Compression deformation amount (mm) | 3.18 | 3.18 | 3.18 | 3.18 | 3.23 |
| Intermediate layer | Formulation No. | c | d | b | c | c |
| | Thickness (mm) | 1 | 1 | 1 | 1 | 1 |
| | Surface hardness Hms (Shore C) | 92 | 83 | 97 | 92 | 92 |
| | Material hardness Hm (Shore D) | 63 | 55 | 68 | 63 | 63 |
| Cover | Formulation No. | f | f | e | f | f |
| | Thickness Tc (mm) | 0.6 | 0.6 | 0.6 | 0.6 | 0.8 |
| | Material hardness Hc (Shore D) | 31 | 31 | 27 | 31 | 31 |
| Dimple | Type (pattern) | V | V | V | VI | V |
| | Lower volume Vi (mm³) | 445 | 445 | 445 | 485 | 445 |
| Golf ball | Surface hardness (Shore C) | 84 | 78 | 87 | 84 | 79 |
| | Compression deformation amount (mm) | 2.78 | 2.86 | 2.7 | 2.81 | 2.81 |
| Hc/Tc×Hm/Vi | | 7.3 | 6.4 | 6.9 | 6.7 | 5.5 |
| Driver shot | Spin rate (rpm) | 2860 | 2920 | 2880 | 2860 | 2990 |
| | Launch angle (°) | 13.3 | 13 | 13.2 | 13.3 | 12.8 |
| | Maximum flying height (m) | 25.1 | 24.8 | 25 | 23.8 | 24.6 |

**Table 7-continued**

| Golf ball No. | | 6 | 7 | 8 | 9 | 10 |
|---|---|---|---|---|---|---|
| Core | Formulation No. | A | A | A | A | A |
| | Diameter (mm) | 39.1 | 39.1 | 39.1 | 39.1 | 39.1 |
| | Surface hardness Hs (Shore C) | 81 | 81 | 81 | 81 | 81 |
| | Compression deformation amount (mm) | 3.23 | 3.23 | 3.23 | 3.23 | 3.23 |
| Intermediate layer | Formulation No. | d | d | d | c | c |
| | Thickness (mm) | 1 | 1 | 1 | 1 | 1 |
| | Surface hardness Hms (Shore C) | 83 | 83 | 83 | 92 | 92 |
| | Material hardness Hm (Shore D) | 55 | 55 | 55 | 63 | 63 |
| Cover | Formulation No. | f | 9 | h | g | f |
| | Thickness Tc (mm) | 0.8 | 0.8 | 0.8 | 0.8 | 0.8 |
| | Material hardness Hc (Shore D) | 31 | 36 | 40 | 36 | 31 |
| Dimple | Type (pattern) | V | V | V | V | IV |
| | Lower volume Vi (mm³) | 445 | 445 | 445 | 445 | 405 |
| Golf ball | Surface hardness (Shore C) | 82 | 74 | 75 | 80 | 79 |
| | Compression deformation amount (mm) | 2.86 | 2.84 | 2.71 | 2.77 | 2.81 |
| Hc/Tc×Hm/Vi | | 4.8 | 5.6 | 6.2 | 6.4 | 6.0 |
| Driver shot | Spin rate (rpm) | 3050 | 3010 | 2930 | 2900 | 2990 |
| | Launch angle (°) | 12.6 | 12.7 | 13 | 13.1 | 12.8 |
| | Maximum flying height (m) | 24.3 | 24.5 | 24.8 | 25 | 25.5 |

**Table 8**

| Golf ball No. | | 11 | 12 | 13 | 14 |
|---|---|---|---|---|---|
| Core | Formulation No. | A | A | A | A |
| | Diameter (mm) | 39.5 | 39.5 | 39.7 | 39.5 |
| | Surface hardness Hs (Shore C) | 81.3 | 81.3 | 81.5 | 81.3 |
| | Compression deformation amount (mm) | 3.18 | 3.18 | 3.14 | 3.18 |
| Intermediate layer | Formulation No. | c | b | b | c |
| | Thickness (mm) | 1 | 1 | 1 | 1 |
| | Surface hardness Hms (Shore C) | 92 | 97 | 97 | 92 |
| | Material hardness Hm (Shore D) | 63 | 68 | 68 | 63 |
| Cover | Formulation No. | f | f | f | 9 |
| | Thickness Tc (mm) | 0.6 | 0.6 | 0.5 | 0.6 |
| | Material hardness Hc (Shore D) | 31 | 31 | 31 | 36 |
| Dimple | Type (pattern) | IV | V | V | IV |
| | Lower volume Vi (mm³) | 405 | 445 | 445 | 405 |
| Golf ball | Surface hardness (Shore C) | 84 | 88 | 90 | 87 |
| | Compression deformation amount (mm) | 2.78 | 2.68 | 2.64 | 2.73 |
| Hc/Tc×Hm/Vi | | 8.0 | 7.9 | 9.5 | 9.3 |
| Driver shot | Spin rate (rpm) | 2860 | 2780 | 2720 | 2800 |
| | Launch angle (°) | 13.3 | 13.7 | 14 | 13.6 |
| | Maximum flying height (m) | 26.4 | 25.7 | 26 | 26.8 |

**Table 8-continued**

| Golf ball No. | | 15 | 16 | 17 | 18 |
|---|---|---|---|---|---|
| Core | Formulation No. | A | A | A | A |
| | Diameter (mm) | 39.1 | 39.5 | 39.5 | 39.1 |
| | Surface hardness Hs (Shore C) | 81 | 81.3 | 81.3 | 81 |
| | Compression deformation amount (mm) | 3.23 | 3.18 | 3.18 | 3.23 |
| Intermediate layer | Formulation No. | a | c | c | c |
| | Thickness (mm) | 1 | 1 | 1 | 1 |
| | Surface hardness Hms (Shore C) | 95 | 92 | 92 | 92 |
| | Material hardness Hm (Shore D) | 66 | 63 | 63 | 63 |
| Cover | Formulation No. | e | f | f | i |
| | Thickness Tc (mm) | 0.8 | 0.6 | 0.6 | 0.8 |
| | Material hardness Hc (Shore D) | 27 | 31 | 31 | 50 |
| Dimple | Type (pattern) | I | II | III | V |
| | Lower volume Vi (mm³) | 285 | 325 | 365 | 445 |
| Golf ball | Surface hardness (Shore C) | 79 | 84 | 84 | 87 |
| | Compression deformation amount (mm) | 2.76 | 2.78 | 2.78 | 2.62 |
| Hc/Tc×Hm/Vi | | 7.8 | 10.0 | 8.9 | 8.8 |
| Driver shot | Spin rate (rpm) | 3020 | 2860 | 2860 | 2600 |
| | Launch angle (°) | 12.7 | 13.3 | 13.3 | 14.5 |
| | Maximum flying height (m) | 27.6 | 28.3 | 27.4 | 26.9 |

The golf ball according to the present disclosure that comprises a spherical core, an intermediate layer positioned outside the spherical core, and an outermost cover positioned outside the intermediate layer and having a plurality of dimples formed thereon, wherein a material hardness Hm (Shore D hardness) of the intermediate layer, a material hardness Hc (Shore D hardness) of the outermost cover, a thickness Tc (mm) of the outermost cover, and a total lower volume Vi (mm³) of the plurality of dimples satisfying Vi>365 and (Hc/Tc)×(Hm/Vi)≤7.5, and wherein a surface hardness in Shore C hardness of the spherical core < a surface hardness in Shore C hardness of the intermediate layer > a surface hardness in Shore C hardness of the golf ball is satisfied, does not have a high maximum flying height in spite of a high spin rate. As a result, the golf ball according to the present disclosure decreases a number of OB shots on a driver shot.

## Claims

1. A golf ball (2) comprising a spherical core (4), an intermediate layer (6) positioned outside the spherical core (4), and an outermost cover (8) positioned outside the intermediate layer (6) and having a plurality of dimples (10) formed thereon, wherein
a material hardness in Shore D hardness Hm of the intermediate layer (6),
a material hardness in Shore D hardness Hc of the outermost cover (8),
a thickness in mm Tc of the outermost cover (8), and
a total lower volume in mm³ Vi of the plurality of dimples (10) satisfy,
Vi>365 and (Hc/Tc)×(Hm/Vi)≤7.5, and wherein
a surface hardness in Shore C hardness of the spherical core (4) < a surface hardness in Shore C hardness of the intermediate layer (6) > a surface hardness in Shore C hardness of the golf ball (2) is satisfied.

2. The golf ball (2) according to claim 1, wherein Vi≥380.

3. The golf ball (2) according to claim 1 or 2, wherein 500≥Vi≥400.

4. The golf ball (2) according to any one of claims 1 to 3, wherein the outermost cover (8) contains a polyurethane as a resin component.

5. The golf ball (2) according to any one of claims 1 to 4, wherein the value (Hc/Tc) is 30 or more and 75 or less.

6. The golf ball (2) according to any one of claims 1 to 5, wherein the value (Hm/Vi) is 0.08 or more and 0.22 or less.

7. The golf ball (2) according to any one of claims 1 to 6, wherein a surface hardness Hs of the spherical core (4) ranges from 60 to 95 in Shore C hardness.

8. The golf ball (2) according to any one of claims 1 to 7, wherein a center hardness Ho of the spherical core (4) ranges from 45 to 74 in Shore C hardness.

9. The golf ball (2) according to any one of claims 1 to 8, wherein the material hardness Hm of the intermediate layer (6) ranges from 50 to 73 in Shore D hardness.

10. The golf ball (2) according to any one of claims 1 to 9, wherein a thickness Tm of the intermediate layer (6) ranges from 0.8 mm to 3.0 mm.

11. The golf ball (2) according to any one of claims 1 to 10, wherein the material hardness Hc of the outermost cover (8) ranges from 20 to 40 in Shore D hardness.

12. The golf ball (2) according to any one of claims 1 to 11, wherein the thickness Tc of the outermost cover (8) ranges from 0.4 mm to 1.0 mm.

13. The golf ball (2) according to any one of claims 1 to 12, wherein a difference (Hms-Hcs) between a surface hardness Hms of the intermediate layer (6) and a surface hardness Hcs of the golf ball (2) is more than 0.

14. The golf ball (2) according to any one of claims 1 to 13, wherein a difference (Hms-Hs) between a surface hardness Hms of the intermediate layer (6) and a surface hardness Hs of the spherical core (4) is more than 0.

## Patentansprüche

1. Golfball (2), umfassend einen kugelförmigen Kern (4), eine Zwischenschicht (6), die außerhalb des kugelförmigen Kerns (4) angeordnet ist, und eine äußerste Abdeckung (8), die außerhalb der Zwischenschicht (6) angeordnet ist und eine Vielzahl von darauf ausgebildeten Vertiefungen (10) aufweist, wobei
eine Materialhärte in Shore-D-Härte Hm der Zwischenschicht (6),
eine Materialhärte in Shore-D-Härte Hc der äußersten Abdeckung (8),
eine Dicke in mm Tc der äußersten Abdeckung (8), und
ein Gesamtvertiefungsvolumen in mm³ Vi der Vielzahl von Vertiefungen (10) erfüllen,
Vi>365 und (Hc/Tc)×(Hm/Vi)≤7,5, und wobei
eine Oberflächenhärte in Shore-C-Härte des kugelförmigen Kerns (4) < eine Oberflächenhärte in Shore-C-Härte der Zwischenschicht (6) > eine Oberflächenhärte in Shore-C-Härte des Golfballs (2) erfüllt ist.

2. Golfball (2) nach Anspruch 1, wobei Vi≥380.

3. Golfball (2) nach Anspruch 1 oder 2, wobei 500≥Vi≥400.

4. Golfball (2) nach einem der Ansprüche 1 bis 3, wobei die äußerste Abdeckung (8) ein Polyurethan als eine Harzkomponente enthält.

5. Golfball (2) nach einem der Ansprüche 1 bis 4, wobei der Wert (Hc/Tc) 30 oder mehr und 75 oder weniger beträgt.

6. Golfball (2) nach einem der Ansprüche 1 bis 5, wobei der Wert (Hm/Vi) 0,08 oder mehr und 0,22 oder weniger beträgt.

7. Golfball (2) nach einem der Ansprüche 1 bis 6, wobei eine Oberflächenhärte Hs des kugelförmigen Kerns (4) in einem Bereich von 60 bis 95 in Shore-C-Härte liegt.

8. Golfball (2) nach einem der Ansprüche 1 bis 7, wobei eine Mittenhärte Ho des kugelförmigen Kerns (4) in einem Bereich von 45 bis 74 in Shore-C-Härte liegt.

9. Golfball (2) nach einem der Ansprüche 1 bis 8, wobei die Materialhärte Hm der Zwischenschicht (6) in einem Bereich von 50 bis 73 in Shore-D-Härte liegt.

10. Golfball (2) nach einem der Ansprüche 1 bis 9, wobei eine Dicke Tm der Zwischenschicht (6) in einem Bereich von 0,8 mm bis 3,0 mm liegt.

11. Golfball (2) nach einem der Ansprüche 1 bis 10, wobei die Materialhärte Hc der äußersten Abdeckung (8) in einem Bereich von 20 bis 40 in Shore-D-Härte liegt.

12. Golfball (2) nach einem der Ansprüche 1 bis 11, wobei die Dicke Tc der äußersten Abdeckung (8) in einem Bereich von 0,4 mm bis 1,0 mm liegt.

13. Golfball (2) nach einem der Ansprüche 1 bis 12, wobei eine Differenz (Hms-Hcs) zwischen einer Oberflächenhärte Hms der Zwischenschicht (6) und einer Oberflächenhärte Hcs des Golfballs (2) mehr als 0 beträgt.

14. Golfball (2) nach einem der Ansprüche 1 bis 13, wobei eine Differenz (Hms-Hs) zwischen einer Oberflächenhärte Hms der Zwischenschicht (6) und einer Oberflächenhärte Hs des kugelförmigen Kerns (4) mehr als 0 beträgt.

## Revendications

1. Balle de golf (2) comprenant un noyau sphérique (4), une couche intermédiaire (6) positionnée à l'extérieur du noyau sphérique (4) et une couverture la plus à l'extérieur (8) positionnée à l'extérieur de la couche intermédiaire (6) et dotée d'une pluralité d'empreintes (10) formées dessus, dans laquelle
une dureté de matériau en dureté Shore D Hm de la couche intermédiaire (6),
une dureté de matériau en dureté Shore D Hc de la couverture la plus à l'extérieur (8),
une épaisseur en mm Tc de la couverture la plus à l'extérieur (8), et
un volume inférieur total en mm³ Vi de la pluralité d'empreintes (10) satisfont,
Vi > 365 et (Hc/Tc) × (Hm/Vi) < 7,5, et dans laquelle
une dureté de surface en dureté Shore C du noyau sphérique (4) < une dureté de surface en dureté Shore C de la couche intermédiaire (6) > une dureté de surface en dureté Shore C de la balle de golf (2) est satisfaite.

2. Balle de golf (2) selon la revendication 1, dans laquelle Vi ≥ 380.

3. Balle de golf (2) selon la revendication 1 ou 2, dans laquelle 500 ≥ Vi ≥ 400.

4. Balle de golf (2) selon l'une quelconque des revendications 1 à 3, dans laquelle la couverture la plus à l'extérieur (8) contient un polyuréthane comme composant de résine.

5. Balle de golf (2) selon l'une quelconque des revendications 1 à 4, dans laquelle la valeur (Hc/Tc) est égale à 30 ou plus et à 75 ou moins.

6. Balle de golf (2) selon l'une quelconque des revendications 1 à 5, dans laquelle la valeur (Hm/Vi) est égale à 0,08 ou plus et à 0,22 ou moins.

7. Balle de golf (2) selon l'une quelconque des revendications 1 à 6, dans laquelle une dureté de surface Hs du noyau sphérique (4) est comprise entre 60 et 95 en dureté Shore C.

8. Balle de golf (2) selon l'une quelconque des revendications 1 à 7, dans laquelle une dureté centrale Ho du noyau sphérique (4) est comprise entre 45 et 74 en dureté Shore C.

9. Balle de golf (2) selon l'une quelconque des revendications 1 à 8, dans laquelle la dureté du matériau Hm de la couche intermédiaire (6) est comprise entre 50 et 73 en dureté Shore D.

10. Balle de golf (2) selon l'une quelconque des revendications 1 à 9, dans laquelle une épaisseur Tm de la couche intermédiaire (6) est comprise entre 0,8 mm et 3,0 mm.

11. Balle de golf (2) selon l'une quelconque des revendications 1 à 10, dans laquelle la dureté du matériau Hc de la couverture la plus à l'extérieur (8) est comprise entre 20 et 40 en dureté Shore D.

12. Balle de golf (2) selon l'une quelconque des revendications 1 à 11, dans laquelle l'épaisseur Tc de la couverture la plus à l'extérieur (8) est comprise entre 0,4 mm et 1,0 mm.

13. Balle de golf (2) selon l'une quelconque des revendications 1 à 12, dans laquelle une différence (Hms - Hcs) entre une dureté de surface Hms de la couche intermédiaire (6) et une dureté de surface Hcs de la balle de golf (2) est supérieure à 0.

14. Balle de golf (2) selon l'une quelconque des revendications 1 à 13, dans laquelle une différence (Hms -Hs) entre une dureté de surface Hms de la couche intermédiaire (6) et une dureté de surface Hs du noyau sphérique (4) est supérieure à 0.
